

B. D. SAKLATWALLA AND A. N. ANDERSON.

PRODUCTION OF REFRACTORY METAL ALLOYS.

APPLICATION FILED APR. 8, 1920.

1,435,742.

Patented Nov. 14, 1922.



By B. D. Saklatwalla  
Arthur N. Anderson  
Bakewell, Bynnes & Partridge  
their Attorneys

## UNITED STATES PATENT OFFICE.

BYRAMJI D. SAKLATWALLA AND ARTHUR N. ANDERSON, OF CRAFTON, PENNSYLVANIA, ASSIGNORS TO VANADIUM CORPORATION OF AMERICA, OF BRIDGEVILLE, PENNSYLVANIA, A CORPORATION OF DELAWARE.

## PRODUCTION OF REFRACtORY METAL ALLOYS.

Application filed April 8, 1920. Serial No. 372,169.

To all whom it may concern:

Be it known that we, BYRAMJI D. SAKLATWALLA and ARTHUR N. ANDERSON, residing at Crafton, in the county of Allegheny and State of Pennsylvania, have invented a new and useful Improvement in the Production of Refractory Metal Alloys, of which the following is a full, clear, and exact description, reference being had to the accompanying drawing, forming part of this specification, in which the figure is a diagrammatic longitudinal vertical section of a furnace designed for carrying out our invention.

15 Our invention relates to the forming of the alloys of highly refractory metals, such as vanadium. Heretofore, it has been considered necessary to use metallic reducing agents, such as silicon or aluminum, in the 20 forming of alloys from ores or materials containing the highly refractory metals.

25 We have discovered a successful, practical process for forming such alloys of vanadium and other high heat refractory metals by the use of carbon as a reducing agent in electric furnace treatment.

In our preferred form of process, there 30 are three factors of importance, which we will now recite in the order of their importance.

1. A critical voltage. We have found it important, if not essential, in commercial manufacture of such alloys of high refractory metals to employ a voltage of one hundred and fifty volts or more with an electric furnace of commercial size; and we have also found that there is a critical current density of at least thirty-five amperes per square inch of cross section of electrodes, we having used a density of from thirty amperes to about ninety amperes per square inch of cross section of electrode. This refers to the alternating current, which we preferably employ.

45 2. Spacing of electrodes where a plurality of electrodes is employed, as in our preferred form. Taking the diameter of an electrode or its thickness in the direction of the next electrode, the spacing between electrodes 50 should lie between 1 and 1.50 of this unit, with the use of the proper resistance of the

bath to regulate the arcs, obtained as hereinafter described.

3. Feeding the charge between the electrodes. By feeding the charge downwardly 55 between the electrodes where a plurality are used, as in our preferred form, the charge is carried directly into the reaction zone and the reduced metal and slag carried away by gravity from that zone and the swirl set up 60 by the effect of the electric current.

By feeding the charge directly into the high temperature reaction zone, the charge is not subject to any substantial preheating or partial reduction previous to its reduction in the high temperature reaction zone. 65 This direct feeding into the high temperature reaction zone is particularly important in smelting vanadium and similar ores in which it is highly desirable that the higher 70 oxides of the ore be reduced directly to the metallic state without preformation of lower oxides.

In all cases, the depending electrode or electrodes should terminate above the level 75 of the metal of the reduced alloy lying below the slag layer, the heat effect being obtained by means of the arc through the charge and through the slag above the metal layer.

Referring now to the drawing, in which 80 we show diagrammatically a preferred form of apparatus for carrying out our invention, 2 represents the metal shell or casing of an electric furnace having a carbon lining 3. This lining may be made of either amorphous or graphitic carbon or both, it being shaped to form a central cavity for the bath. Above the lining is a refractory cover 4, preferably formed of refractory brick, with water-cooling devices embedded therein, 85 through which water is circulated. This refractory cover is provided with a hole or holes, preferably lined with annular water-cooling devices, indicated at 5, through which depend the electrodes 6, which fit 90 closely therein, the furnace chamber being preferably substantially air-tight. In the form shown, there are three electrodes each connected to the lines 7 of a three-phase alternating current supply, which is above one 95 hundred and fifty volts and of high current density, as above recited. The electrodes are 100

preferably circular in cross section, although they may be of other shapes.

Between the electrodes and extending through holes in the refractory cover are 5 feed chutes 8, through which the charge is fed by gravity, preferably in a continuous manner, to the region or regions between the electrodes. The electrodes may be arranged, as shown, or may be arranged at the corners 10 of a triangle, preferably an equilateral triangle. In the latter case, a single feed chute could be used at the center of the triangle, discharging into the region between the electrodes. 15 The drawing illustrates diagrammatically the layers of materials as in regular operation, and the temperature zone. Thus, A represents the lower layer of molten alloy which may be tapped out from time to time 20 through the tap hole 9. The outer portions A' of this layer are shown as congealed or partly congealed. Above this molten metal layer is the layer B of slag with the charges entering it between the electrodes, as indicated. 25 This slag zone is shown as having a dished or concave surface, which is somewhat exaggerated in the drawing. This surface is due to the swirling or whirlpool action of the molten bath or the upper portion thereof, 30 resulting from the action of the electric current, and it will be noted that the charge feed is into the central portion of this swirl. The dotted lines X—X indicate the zone of highest temperature under the conditions 35 shown, within which zone the reducing action takes place, this temperature zone being surrounded by the outer slag annulus B'.

In forming a vanadium alloy, the charge is a mixture of pulverized vanadium ore, or 40 vanadium-bearing material, such as vanadium oxide or sulphide, iron, preferably in the form of iron scale or iron ore, and fluxes, such as glass cullet, lime, fluorspar and coke. The glass cullet or similar flux has two important 45 functions: 1st, to increase the electric resistance; and second, to control the speed of the whirl by increasing the viscosity of the slag, and thus reducing the washing effect on the lining. The iron scale also serves 50 to increase the electric resistance, and hence serves to regulate the length and localization of the arc; and also as it is reduced, forms the alloy of ferro-vanadium desired. The commercial ferro-vanadium product now in 55 demand contains about 30% to 40% of vanadium, and we have made such alloys as high as 50% vanadium.

As an example of the mix under the conditions herein recited, we have used from one 60 to five per cent of cullet and from two per cent of iron scale for low grade ore up to fifteen per cent for high grade ore, coke also being added.

In case the gangue constituents of ore or 65 vanadium-containing material have fluxes

and constituents somewhat similar to that of glass cullet, the cullet need not be added. These percentages will depend to a considerable extent upon the chemical composition of the ore or vanadium-bearing material. 70

Under the conditions shown and recited, taking the electrode diameter as a unit, the distance between electrodes is about 1.25. The distance from the outer electrodes to the edge of the bath is shown as 2 and may 75 vary from 2 to 3, and the over-all diameter of the bath is about 9.50, the current being over 150 volts and with a density of between 35 and 50 amperes per square inch of electrodes in cross section. The slag may be 80 drawn off through the slag tap 10. As the operation goes on, the entering charges fed in between the electrodes enter the best zone of reduction and are drawn down by the swirling action. The ends of the electrodes 85 lie in the slag layer above the metal layer, and reduction is rapid and effective under the conditions named. We have found that vanadium reduction demands a very high 90 temperature, a quick reaction and a quick removal from the zone of reaction. The reaction is highly localized by something like a blow-pipe effect. The drawing is scaled to the preferred relative areas employed under the conditions named as to voltage and density, character of mix, arrangement of electrodes, with three-phase current, etc. 95

The current is preferably controlled by a control system, such as that shown, for example, in our co-pending applications, Serial Nos. 292,285 and 292,286, filed April 24, 1918. The alloy formed contains about 30 to 40% of vanadium, the remainder being iron with certain metals or metalloids, such as silicon, manganese and carbon. 100

The advantages of our invention will be apparent to those skilled in the art, since we believe that we are the first to attain the production of vanadium alloys without the use of metallic reducing agents. A reduction 110 of carbon has been desired, and has been attained by us by means of the process above recited.

The important features of the process may be carried out with less efficiency, however, 115 by the use of a single electrode, or upper and lower electrodes with a single or multiphase current. If a single electrode is used, the current should be at least 150 volts and above the lower amperage limit of 35 amperes, per 120 square inch of electrode. In such case, the feed should be as nearly as possible to the base of the electrode.

The vanadium-bearing material may be varied, the form of carbon used may be 125 changed, the fluxes may be varied so long as proper electrical resistance to regulate the arc is obtained in the slag layer, the number and arrangement of the electrodes may be changed, and other variations may be made, 130

without departing from our invention, as defined in the broader claims.

We claim:

1. In the method of forming alloys of highly refractory metals, the steps consisting of reducing the metal in an electric furnace under a voltage of more than 150 volts, substantially as described.
2. In the method of forming alloys of highly refractory metals, the steps consisting of reducing the metal in an electric furnace under a voltage of more than 150 volts and of at least 35 amperes per square inch of electrode area, substantially as described.
3. In the method of forming alloys of highly refractory metals, the steps consisting of feeding charge material into a plural electrode furnace having a spacing between the electrodes of 1 to 1.5, based on the thickness of an electrode as a unit, substantially as described.
4. In the method of forming alloys of highly refractory metals, the steps consisting of feeding charge material into an electric furnace having an electric current supply of at least 150 volts and of high current density, with a spacing between the electrodes of 1 to 1.5 based on the thickness of an electrode as a unit, substantially as described.
5. In the herein described method, the steps which consist in maintaining in the hearth of an electric furnace a molten bath into which the furnace electrodes extend and produce between them a high temperature reaction zone, and in feeding directly into such reaction zone highly refractory metal-bearing material and carbonaceous material, substantially as described.
6. In the method of forming alloys of highly refractory material, the steps consisting of feeding a charge in the region between a plurality of electrodes of an electric furnace, and supplying current to the electrodes of at least 150 volts, substantially as described.
7. In the method of forming alloys of highly refractory material, the steps consisting of feeding a charge in the region between a plurality of electrodes of an electric furnace, and supplying current to the electrodes of at least 150 volts and at least 35 amperes per square inch of electrodes, substantially as described.
8. In the herein described method, the steps which consist in maintaining in the hearth of an electric furnace a molten bath having a slag layer into which the furnace electrodes extend and produce between them a high temperature reaction zone, and in feeding directly into such reaction zone highly refractory metal-bearing material and carbonaceous material, substantially as described.
9. In the method of forming alloys of highly refractory material, the steps consist-
10. In the method of forming alloys of highly refractory material, the steps consisting of feeding charge-forming material downwardly between the electrodes of a plural-electrode furnace having a spacing between the electrodes of 1 to 1.5 based on the thickness of the electrode as a unit, and supplying a current of at least 150 volts, substantially as described.
11. In the method of forming alloys of highly refractory material, the steps consisting of feeding into the region between the electrodes of a plural-electrode furnace a mixture of vanadium-containing material, alloying material and carbonaceous material, and supplying to the electrodes a current of at least 150 volts with a capacity of at least 35 amperes per square inch of electrodes, substantially as described.
12. In the method of forming alloys of highly refractory material, the steps consisting of feeding into the region between the electrodes of a plural-electrode furnace a mixture of vanadium-containing material, alloying material and carbonaceous material, and supplying to the electrodes a current of at least 150 volts with a capacity of at least 35 amperes per square inch of electrodes, the electrodes being spaced apart from 1 to 1.5 based on the thickness of an electrode as a unit, substantially as described.
13. In the method of forming alloys of highly refractory material, the steps consisting of maintaining a lower bath of molten alloy with an upper layer of slag in a plural-electrode furnace, feeding a mixture containing vanadium-bearing material into the region between the electrodes which terminate above the molten metal layer, and supplying a current of at least 150 volts, substantially as described.
14. In the method of forming alloys of highly refractory material, the steps consisting of maintaining a lower bath of molten alloy with an upper layer of slag in a plural-electrode furnace, feeding a mixture containing vanadium-bearing material into the region between the electrodes which terminate above the molten metal layer, and supplying a current of at least 150 volts and at least 35 amperes per square inch of electrodes, substantially as described.
15. In the method of forming alloys of highly refractory material, the steps consisting of maintaining a lower bath of molten alloy with an upper layer of slag in a plural-electrode furnace, feeding a mixture containing vanadium-bearing material into the

region between the electrodes which terminate above the molten metal layer, and supplying a current of at least 150 volts and at least 35 amperes per square inch of electrodes, the electrodes being spaced apart a distance greater than the thickness of an electrode as a unit, substantially as described.

16. In the herein described method, the step which consists in feeding a mixture containing vanadium-bearing material and carbonaceous material directly into the high temperature reaction zone of an electric smelting furnace, substantially as described.

17. In the herein described method, the step which consists in feeding a mixture containing a vanadium-bearing material, a fluxing material, and carbonaceous material directly into the high temperature reaction zone of an electric smelting furnace, substantially as described.

18. In the herein described method, the step which consists in feeding a mixture containing a vanadium-bearing material, an alloying metal-bearing material, and carbonaceous material directly into the high temperature reaction zone of an electric smelting furnace, substantially as described.

19. The method of reducing vanadium containing materials, which consists in maintaining in the hearth of an electric furnace a molten bath into which the furnace electrodes extend and produce between them a high temperature reaction zone, and in feeding directly into such reaction zone a vanadium containing material and carbonaceous material, substantially as described.

20. The method of reducing vanadium-containing materials, which consists in electrically smelting such materials to the metallic state with a carbonaceous reducing agent, substantially as described.

21. The method of reducing vanadium-containing materials, which consists in smelting such materials to the metallic state with a carbonaceous reducing agent, substantially as described.

22. The method of making ferro-vanadium, which consists in electrically smelting iron and vanadium-containing materials to the metallic state with a carbonaceous reducing agent, substantially as described.

23. The method of reducing vanadium-containing materials, which consists in maintaining in the hearth of an electric furnace a molten bath having a slag layer into which the furnace electrodes extend and produce between them a high temperature reaction zone, and in feeding directly into such

reaction zone a vanadium-containing material and carbonaceous material, substantially as described.

24. The method of reducing vanadium-containing materials, which consists in maintaining in the hearth of a furnace a molten bath having a localized high temperature reaction zone, and in feeding directly into such reaction zone a vanadium-containing material and carbonaceous material, substantially as described.

25. The method of reducing vanadium-containing materials, which consists in maintaining in the hearth of a furnace a molten bath having a localized high temperature reaction zone, in feeding directly into such reaction zone a vanadium-containing material and carbonaceous material, holding the materials in such zone until the vanadium is reduced to the metallic state, and removing the reduced vanadium metal from such zone by gravity, substantially as described.

26. The method of making ferro-vanadium, which consists in maintaining in the hearth of a furnace a molten bath having a localized high temperature reaction zone, and in feeding directly into such reaction zone iron and vanadium-containing materials and carbonaceous material, substantially as described.

27. The method of making ferro-vanadium, which consists in maintaining in the hearth of a furnace a molten bath having a localized high temperature reaction zone, in feeding directly into such reaction zone iron and vanadium-containing materials and carbonaceous material, holding the materials in such zone until the vanadium and iron are reduced to metallic ferro-vanadium, and removing the reduced ferro-vanadium metal from such zone by gravity, substantially as described.

28. The method of reducing vanadium-containing materials, which consists in smelting such materials to the metallic state with a carbonaceous material and a fluxing material, substantially as described.

29. The method of making ferro-vanadium, which consists in smelting iron and vanadium-containing materials to the metallic state with a carbonaceous reducing agent and a fluxing material, substantially as described.

In testimony whereof, we have hereunto set our hands.

BY RAMJI D. SAKLATWALLA.  
ARTHUR N. ANDERSON.